

Aug. 19, 1941.

B. E. L. DE MARÉ

2,253,421

METHOD AND APPARATUS FOR DEOXIDIZING AND DEGASIFYING LIQUID STEEL

Filed Sept. 18, 1939



Inventor  
Baltzar E. L. de Maré  
by his Attorneys  
Sorenson & Sorenson

## UNITED STATES PATENT OFFICE

2,253,421

## METHOD AND APPARATUS FOR DEOXIDIZING AND DEGASIFYING LIQUID STEEL

Baltzar E. L. de Maré, Philadelphia, Pa.

Application September 18, 1939, Serial No. 295,491  
In Sweden September 20, 1938

3 Claims. (Cl. 75—13)

This invention relates to the treatment of liquid steel, to improve the quality thereof by eliminating the two chief causes of defects in articles formed therefrom, namely the elimination of products of oxidation, chiefly silicates of manganese and aluminum which cause non-metallic impurities in the articles; and the elimination of occluded gases, such as hydrogen, nitrogen and carbon monoxide which cause seams.

The object of the invention is to provide a thoroughly practical method for such treatment, to replace methods hitherto known or proposed which have proven to be, in one or more respects, commercially impractical, inefficient, or unadaptable and have therefore been discarded.

For instance, it has previously been proposed to pour molten metal into a mould placed in an air-evacuated chamber, to give the vacuum a chance to eliminate gases occluded in the metal. Thus, for instance, a whole electric furnace and one or more moulds have been placed under one large bell for evacuation. The bell therefore, was necessarily large in size, heavy, and unwieldy. Incidentally, the means for handling the furnace and the mould, or moulds, were complicated and expensive.

It has also been proposed to arrange the moulds alone, with a distributing arrangement for the metal, in a vacuum chamber, and to employ a special ladle as a cover for the chamber, above the distributing arrangement. This arrangement is necessarily difficult to handle, bulky, and complicated and suffers further from the disadvantage that the evacuation of the vacuum chamber cannot begin until the ladle has been placed in position.

Normally the pouring of liquid metal directly into a mould under vacuum involves the disadvantage that the metal, upon making contact with the cast iron mould, chills rapidly and solidifies before the vacuum can become effective to extract all the occluded gases and before the slag and impurities can be carried upwards by the gases to the top of the ingot being formed in the mould.

It has been proposed to provide a ladle or similar receptacle with a tight cover connected with an evacuating arrangement, and on this cover to place a receptacle from which liquid metal contained therein may be poured into the ladle. This arrangement has the disadvantages that the ladle must be specially constructed; that the ladle must be provided with air-tight surfaces at its top; and that the cover cannot be removed without

out breaking the connection with the evacuating arrangement.

Both of the last named arrangements have an additional disadvantage in that the ladle in which 5 the vacuum treatment is being carried out is surrounded by air, therefore the radiation of heat from the ladle becomes considerable. For that reason the metal cannot be permitted to remain for any prolonged period of time in the ladle. 10 Therefore, the vacuum treatment cannot be continued for a sufficient length of time to be thoroughly effective.

It has also been proposed to treat the liquid metal with deoxidizing slag to remove oxides and 15 other impurities from the metal, by causing the metal to fall from a great height into a receptacle containing such slag, to cause a violent impact therebetween for creating an intermixing of the two. This involves the disadvantage 20 that oxidization of the metal and loss of heat by radiation and convection increase in proportion to the height of its fall.

The several disadvantages pointed out above in 25 regard to the heretofore known methods and arrangements are avoided in the invention at hand, according to which the treatment can be carried out in a practical way by the use of ordinary ladles and with the greatest possible effectiveness.

The present invention also ensures that the 30 pouring can be done conveniently in the usual way and under atmospheric pressure, after the deoxidizing and degasifying treatment has been finished.

The present invention is chiefly distinguished 35 from the prior art in that the liquid metal, tapped from a converter or melting furnace into a ladle, is poured from said ladle into a smaller open vessel or pouring box arranged the shortest possible distance below the ladle and having controlled communication with a vacuum chamber; in that the metal, while in this vessel is subjected to electric heating and cleaning by a suitable deoxidizing slag; in that the liquid metal 40 is permitted to flow from this vessel in a stream down into a ladle removably enclosed in the vacuum chamber; in that during its pouring into the enclosed ladle the liquid metal is exposed to the action of a high vacuum; in that after the pouring is completed the exposure of the 45 liquid metal to said high vacuum is continued for a desired period of time; and in that the last named ladle, after the vacuum treatment has been finished and atmospheric pressure restored, is taken out of the vacuum chamber and its content poured off into moulds. Further distinc-

tive features and advantages of the invention will be made evident by the following description and appended claims.

In the accompanying drawing is shown a design of an arrangement for carrying out the method according to the invention, the single figure of the drawing being a vertical section of the preferred arrangement for the vacuum treatment of liquid steel.

In the drawing, 1 denotes a vacuum chamber formed within a suitable structure placed in the ground, such as a concrete pit 2, which may be reinforced with an outer air-tight casing 3, and provided with a refractory lining, as shown at 4.

The vacuum chamber 1 is covered with a convex lid 5, which is provided with a suitable heat-insulating lining, for instance concrete, and with lifting clevises 6 for the handling thereof. The lid 5, at its under edge, is provided with a labyrinth packing 7, which consists of a number of concentric ridges with sharp edges, which edges rest on a machine finish bottom of a trough-shaped channel 8 covered with a suitable plastic material into which said edges are pressed. The sloping inside wall 9 of the trough 8 forms a frusto-conical guide for the lid 5.

On the lid 5, a small open vessel or pouring box 10 is mounted and suitably secured. The vessel 10 communicates with the vacuum chamber 1 through a nozzle 11 disposed in the bottom of the vessel 10. The opening or hole of the nozzle 11 can be closed or opened by means of a stopper rod 12. The entrance of air into the vacuum chamber 1 is at first prevented by the stopper 12 and after the level of the metal in the vessel 10 is raised to a predetermined height the liquid metal in the vessel 10 forms the necessary seal.

In the construction shown, the vessel 10 is surrounded by an electric coil 13 and is designed as a high frequency electric furnace of the Northrup type, for example.

The lid 5 of the vacuum chamber 1 can be provided with an air-admission valve 25 and a sight glass 30 for observation and for use of an optical pyrometer for determining the temperature of the stream 28 in comparison to the temperature of the stream 24, also determined by optical pyrometer, or with other arrangements, by which the course of treatment in the vacuum chamber 1 can be regulated or controlled, and according to which the strength of the electric current in coil 13 can be suitably regulated.

A ladle 16 is shown above the vessel 10, by which ladle the liquid steel is carried from the converter or melting furnace to the vacuum apparatus, 17 denotes the removable ladle in the vacuum chamber 1, into which the metal is poured and in which the treated metal is collected as the vacuum treatment is being carried out. Both the ladles 16 and 17 can be constructed identically, so that exchanges can be made.

In the vacuum chamber 1, there is a plurality of supports or piers 18, which are provided with conically shaped attachments 19 to serve as guides and supports for the ladles and which co-operate with attachments 20 on the ladles for that purpose. The ladles may be provided with an insulating space between the outside plate shell and the lining of the ladle. The ladles are also provided with stopper rods 22 for controlling the flow of the liquid steel through the nozzles 23.

The vacuum chamber 1 is connected by means of a heavy duty pipe 27 and pipe-fitting assembly with any suitable air evacuating apparatus, for

instance, a steam-jet air-ejector of such capacity as to quickly evacuate the vacuum chamber and reduce the pressure in the vacuum chamber to a minimum low value, approximating zero.

The vacuum treatment is carried out in the following way: Liquid steel from a "Bessemer" converter, or melting furnace is tapped into the ladle 16, which is then taken to and supported above the vessel 10. The liquid steel is permitted to flow through the nozzle 23 of the ladle 16 into the vessel 10. The nozzle 11 in the bottom of the vessel 10 is opened, after the vessel 10 has been filled to a suitable height with liquid steel. From the vessel 10, the steel is permitted to flow as a stream 28 into the preheated ladle 17 in the vacuum chamber 1.

The metal in the stream 28 will, during its passage through the vacuum chamber 1, previously evacuated, become degasified, and the degasification continues afterwards with respect to the liquid mass of steel 29 which collects in the ladle 17.

In the vessel 10 may be added preheated or melted slag 15, as for instance an acid reducing slag or any other suitable kind of slag, by which the liquid steel undergoing treatment may be acted on and purified. The slag 15 also protects the steel against oxidation and radiation of heat. The slag 15 is heated and melted to a substantially liquid state prior to being placed in the vessel 10, such preheating and melting being accomplished by any suitable means forming no part of the present invention.

With the arrangement as shown, an electric heating of the steel may be effected while passing through the vessel 10. For this purpose the vessel 10 is designed as an open high frequency electric furnace. All of the metal from the ladle 16 is cleansed while passing through the vessel 10, by being brought into intimate contact with the slag 15 under a circulating action created in the metal by the heating electric current.

In the present instance, the capacity of the electric furnace 10 is substantially one-tenth the capacity of the furnace or converter from which the liquid metal is drawn into the ladle 16 for pouring into the vessel 10.

After the pouring of the steel into the ladle 17 has been finished, and the deoxidizing slag in the vessel 10 has also been drained off into the ladle 17, the nozzle 11 is closed tightly by the stopper 12 to preserve the vacuum in the chamber 1, to allow for further vacuum treatment of the steel, and after degasification and deoxidization of the metal has been continued for the desired length of time, air is admitted into the vacuum chamber, the lid 5 is removed and the ladle 17 is hoisted out of the chamber 1 and taken to the place where the pouring of the steel into the moulds is to be done.

As it leaves the nozzle 11 of the pouring box 10, through the sudden release of the gases as the metal enters the vacuum chamber 1, the stream 28 of liquid steel may assume the form of a spray, providing quicker and greater liberation of the occluded gases.

While the metal is held under the vacuum in the ladle 17, the minute particles of the impurities coalesce and move upward to and collect at the top of the static body of metal in the ladle 17. By being able to hold the metal in a liquid state in the ladle 17 within the vacuum chamber 1 for a considerable length of time, the impuri-

ties are given ample opportunity to rise to the top.

The carrying out of the method as described above is, of course, to be considered as an example and the invention can be modified in different ways within the scope of the appended claims.

The process according to the invention can naturally be applied to the treatment of metals other than steel. The apparatus shown admits of many varying possibilities for the treatment of liquid metals.

In addition to the dynamic and static vacuum treatment described above, the apparatus may be used for only static vacuum treatment, and the electrical arrangements shown may be used simply for superheating the metal. Should, for instance, the metal in the ladle 17, after the vacuum treatment, be too cold, the ladle 17 may be hoisted and the empty ladle 16, or another similar ladle, placed in the vacuum chamber, and by again pouring the metal through the vessel 10 the temperature of the metal may be raised to the desired degree by means of the electric heating arrangements.

I claim:

1. Method to deoxidize and degasify liquid steel, characterized by the liquid steel being tapped into a ladle from a Bessemer converter or melting furnace, being then poured from said ladle through a smaller open vessel into a ladle located in a vacuum chamber, wherein the metal during its passage through said vessel is electrically heated and brought into intimate contact with a deoxidizing slag by action of the electric

heating currents, and wherein the metal during its passage from said vessel to the ladle in the vacuum chamber is subjected to high vacuum to effect degasifying of the metal.

2. Method to deoxidize and degasify liquid steel, characterized by the liquid steel being tapped into a ladle from a Bessemer converter or melting furnace, being then poured from said ladle through a smaller open vessel into a ladle located in a vacuum chamber, wherein the metal during its passage through said vessel is electrically heated and brought into intimate contact with a deoxidizing slag by action of the electric heating currents, wherein the metal during its passage from said vessel to the ladle in the vacuum chamber is subjected to high vacuum to effect degasifying of the metal, and wherein the vacuum treatment is continued after the pouring of the metal into the ladle in the vacuum chamber has stopped to continue said degasifying and to permit the impurities to rise to the top of the metal.

3. An apparatus for the treatment of liquid steel, comprising a vacuum chamber, a ladle in said chamber, a ladle outside and above said chamber, an open vessel between said ladles and in direct communication with the interior of said vacuum chamber, electric means for heating the liquid steel poured from the outside ladle through said pouring box into the ladle within the vacuum chamber, and means for drawing a high vacuum in said chamber to effect said treatment of said liquid steel.

BALTZAR E. L. DE MARÉ.